

May 30, 1950

F. BROCKMAN  
ELECTRICAL CONDENSER

2,509,758

Filed Jan. 26, 1949



FIG. 1



FIG. 2

FRANK BROCKMAN  
INVENTOR

AGENT

## UNITED STATES PATENT OFFICE

2,509,758

## ELECTRICAL CONDENSER

Frank Brockman, Dobbs Ferry, N. Y., assignor to  
 Philips Laboratories, Inc., Irvington on Hudson,  
 N. Y.

Application January 26, 1949, Serial No. 72,959

8 Claims. (Cl. 175—41)

1

My invention relates to electrical condensers. It is an object of my invention to provide a new and novel electrical condenser.

It is a further object of my invention to provide a temperature responsive electrical condenser having improved characteristics.

These and further objects of my invention will appear as the specification progresses.

The electrical condenser according to my invention comprises two electrodes and a dielectric of a ferromagnetic core material consisting essentially of mixed crystal ferrites of selected metal oxides. Such materials, which are described in the U. S. Patents 2,452,529; 2,452,530 and 2,452,531 dated October 26, 1948 to J. L. Snoek, consist of mixed crystals of a plurality of oxides of bivalent materials mixed and reacted with iron oxide.

Electrical condensers according to my invention exhibit an unexpectedly high capacitance for a given size, and I have found that this is due to the fact that such materials have unexpectedly high dielectric constants which are greater than 100 and in some instances of the order of  $10^4$  to  $10^5$ . In addition, my electrical condensers have the further advantage that they have a large absolute variation capacity with changes in temperature and I have found that this is due to the unusual temperature dependence of the dielectric constant of such materials.

In order that the invention may be more clearly understood and carried into effect, it will now be described with reference to the accompanying drawing in which:

Fig. 1 is a curve indicating the dependence of the dielectric constant of the dielectric on temperature; and

Fig. 2 is a capacitor according to the invention.

Referring to the drawing, I have shown in Fig. 1 the temperature dependence of the dielectric constant of a particular mixed crystal ferrite, i. e., manganese-zinc ferrite the constituent components of which consist for example of about 23 mol per cent manganese oxide, about 25 mol per cent zinc oxide and about 52 mol per cent iron oxide. Although the invention will be described with reference to this particular material, I wish it to be understood that other mixed crystal ferrites described in the above-identified patents are suitable for the invention, e. g. copper-zinc ferrite, magnesium-zinc ferrite, copper-cadmium ferrite and nickel-zinc ferrite.

Referring to Fig. 1, the ordinates are specified in values of the dielectric constant  $E$  and the abscissae in degrees centigrade of temperature.

2

It should be noted that the curve is a measure of the real part of the dielectric constant, an imaginary part not being shown since it in no way influences the character of the invention. 5 To those familiar in the art, it is known that at higher frequencies, e. g. above one megacycle, the true dielectric constant of a material is composed of a real part and imaginary component corresponding to the real and imaginary parts 10 of a complex argument of a mathematical function.

It will be seen from the curve that the dielectric constant at temperatures below the temperature indicated as the magnetic Curie point, has a value of the order of  $10^5$  and gradually 15 decreases until it nears the magnetic Curie temperature. In the neighborhood of the magnetic Curie temperature, the dielectric constant decreases rapidly. Quite unexpectedly I found 20 that in the vicinity of the magnetic Curie temperature the dielectric constant rises very sharply and levels off at a lower value than the initial value of the dielectric constant at the start of the curve.

25 The Curie point of a magnetic material is that temperature above which the magnetic material has a negligible permeability and for all practical purposes is no longer ferromagnetic. The Curie point of ferromagnetic mixed crystal ferrite 30 materials to which the present invention is directed can be controlled over a wide range of temperatures as set forth in the above noted patents and therefore the temperature at which the dielectric constant of the materials exhibits 35 a sharp drop in value as well as the slope of the change in dielectric constant with temperature over a given operating temperature range can similarly be controlled.

The condenser shown in Fig. 2 comprises a dielectric 1 in the form of a disc and consisting 40 essentially of a mixed crystal ferrite as above described and electrodes 2—2 consisting for example of metal layers of silver, copper, gold, lead, tin or the like positioned on the dielectric by spraying, firing or the like. When utilizing as 45 a dielectric the manganese-zinc ferrite above specifically described, the condenser exhibits a negative temperature coefficient of capacity over the temperature range below the magnetic Curie point, i. e. over the temperature range between 50 20° and 150° C. At the magnetic Curie temperature a sharp reversal in the temperature coefficient occurs and within a temperature change of approximately one degree a large change in 55 capacitance occurs.

Such capacitors would be useful for numerous applications. For example, the capacitor described is useful in radio circuits as a temperature compensating capacitor for correcting undesirable frequency drift due to temperature changes of the circuit components. Furthermore the capacitor is suitable as a temperature responsive switch because of the abrupt change in capacitance over a small temperature range i. e. of the order of 1° C., which it undergoes at temperatures about the magnetic Curie point.

Where a large capacitance per unit volume is desired, the unexpectedly high dielectric constant of the material makes these condensers particularly useful.

As above noted the magnetic Curie temperature of the ferrites can be controlled to any desired value as described by J. L. Snoek in the above-identified patents which therefore renders possible capacitors of varying characteristics each suited to a particular desired application.

While I have thus described my invention with specific examples and applications, I do not wish to be limited solely thereto as other modifications will be apparent to those skilled in the art without departing from the spirit and scope of the invention.

What I claim is:

1. An electrical condenser comprising a pair of electrodes and a dielectric therebetween consisting essentially of a mixed spinel crystal ferrite material.
2. An electrical condenser comprising a pair of electrodes and a dielectric therebetween consisting essentially of a ferromagnetic mixed spinel crystal ferrite material.
3. An electrical condenser comprising a pair of electrodes and a dielectric therebetween consisting essentially of a ferromagnetic mixed spinel crystal ferrite material having a dielectric constant greater than 100.
4. An electrical condenser comprising a pair of electrodes and a dielectric therebetween consist-

ing essentially of a ferromagnetic mixed spinel crystal ferrite material having a dielectric constant of the order of  $10^5$ .

5. An electrical condenser comprising a pair of electrodes and a dielectric therebetween consisting essentially of mixed crystals of manganese-zinc ferrite having a dielectric constant of the order of  $10^5$ .

10 6. An electrical condenser comprising a pair of electrodes and a dielectric therebetween consisting essentially of mixed crystals of manganese-zinc ferrite, said dielectric having a magnetic Curie point within the normal operating range of temperatures of the condenser and having a dielectric constant of the order of  $10^5$ .

15 7. An electrical condenser comprising a pair of electrodes and a dielectric therebetween consisting essentially of mixed crystals of manganese-zinc ferrite, said dielectric having a magnetic Curie point at about 160° C. and having a dielectric constant of the order of  $10^5$ .

20 8. An electrical condenser comprising a pair of electrodes and a dielectric therebetween consisting essentially of mixed crystals of manganese-zinc ferrite, said dielectric having a magnetic Curie point at about 160° C. and exhibiting a sharp rise in the value of the dielectric constant at the said temperature, said dielectric having a dielectric constant of the order of  $10^5$ .

FRANK BROCKMAN.

#### REFERENCES CITED

The following references are of record in the file of this patent:

#### UNITED STATES PATENTS

| Number    | Name    | Date          |
|-----------|---------|---------------|
| 2,306,555 | Mueller | Dec. 29, 1942 |
| 2,443,094 | Carlson | June 8, 1948  |
| 2,452,529 | Snoek   | Oct. 26, 1948 |
| 2,452,530 | Snoek   | Oct. 26, 1948 |